

## UNITED STATES PATENT OFFICE

2,197,712

MINERAL OIL COMPOSITIONS AND PROC-  
ESSES OF PREPARING THE SAMEAnderson W. Ralston and Everett J. Hoffman,  
Chicago, Ill., assignors to Armour and Com-  
pany, Chicago, Ill., a corporation of IllinoisNo Drawing. Application October 14, 1938  
Serial No. 235,094

7 Claims. (Cl. 87—9)

This invention relates to mineral oil compositions and processes of preparing the same, and it comprises mineral oil compositions, such as lubricating oils and greases, containing small amounts of an acylated and polymerized coumarone, it further comprises such mineral oil compositions containing small amounts of the product of acylating coumarone, or one of its polymers, in the presence of a metallic chloride acylating catalyst, hydrolyzing the intermediate metallic chloride complex and recovering the catalyst-free acylated and polymerized coumarone.

For many uses in the art lubricating oil compositions having low pour points must be used. The pour point of an oil is in part directly related to the amount of paraffin wax in the oil and it is customary to dewax the oil both for the recovery of usable paraffin and for lowering the pour points of the oil. Even after drastic dewaxing operations the final lubricating oil does not always have as low a pour point as the art desires. Paraffin wax itself, however, has lubricating characteristics, and prior workers have sought to keep some of the wax in the oil by so modifying the pour point of the oil that in spite of its wax content the oil can be used for lubricating at low temperatures. This has been accomplished in recent years by adding to the oil substances to which the name "pour point depressors" has been given. Quite a few substances for this purpose have been discovered. Theoretically it is assumed that a pour point depressor inhibits crystallization of the paraffin wax in the oil and thus prevents the oil, when subjected to low temperatures, from forming a kind of sludge or slush of relatively large wax crystals occupying the entire volume of the oil and occluding liquid oil within the network of crystals.

At the present time condensation products between chlorinated paraffins and aromatics are used to a considerable extent as pour point depressors. Products of this nature are much less effective in their actions than compounds described in this invention. In addition they contribute nothing to the oiliness of the lubricant to which they are added, which is markedly different from our products.

In all instances the amount of pour point depressor added is relatively small. The quantities generally average a fraction of a percent based on the quantity of oil.

We have now discovered a class of materials

which function particularly well as pour point depressors, and which have the added advantage that they impart oiliness to the oil. The substances which we use can be generically defined as acylated coumarones wherein the acyl group contains at least twelve carbon atoms. These acylated coumarones are new materials in themselves and are the subject matter of the Ralston, Vander Wal and Segebrecht application Serial No. 228, 261, filed September 2, 1938. These compounds are prepared, broadly speaking, by reacting coumarone, or one of its polymers, with a fatty acid chloride having at least twelve carbon atoms in the presence of an acylating catalyst, such as aluminum chloride. This reaction results in the formation of an intermediate complex containing the catalyst which is thereafter hydrolyzed to free it of catalyst, and the final product recovered. Thus the preparation of these acylated coumarones follows closely the acylation of other aromatic hydrocarbons by the Friedel-Crafts synthesis. But during the acylation of the coumarone the coumarone polymerizes. Or it is possible that the coumarone is first acylated and thereafter the acyl derivative polymerizes. In any event, the final product is an acylated and polymerized coumarone. Or, to put it more definitely, it is a polymerized coumarone containing acyl groups having twelve or more carbon atoms.

In the preparation of these pour point depressors any fatty acid chloride having twelve or more carbon atoms can be used. These can be either saturated or unsaturated, or they can be fatty acid chlorides made from fatty acids prepared by the oxidation of paraffin wax or other hydrocarbons yielding fatty acids on oxidation. Mixtures of two or more different fatty acid chlorides can be used as the acylating agent. This gives us final products of mixed character and very complex constitution. Indeed the pour point depressor effect of our products may possibly be due to the complex nature of them. As fatty acid chlorides we can use lauryl, myristyl, palmityl, stearyl, oleyl, linoleyl and linolenyl chlorides, these being the more usual ones.

In broad aspects, the fatty acid chloride is added to a suspension of the acylating catalyst, such as aluminum chloride, in an inert solvent, and to this mixture coumarone dissolved in an inert solvent is added. The proportions of fatty acid chloride to coumarone can vary over wide limits as we have found by experiment. This probably means that so long as the coumarone

polymer contains at least one acyl group the product has pour point depressor characteristics. But more than one acyl group can be present in the final product.

We shall now give an example of how our pour point depressors are made from fatty acid chlorides of at least twelve carbon atoms and coumarones.

*Example*

10. Twenty grams of aluminum chloride are suspended in 50 cc. of tetrachloroethane in a three-necked flask equipped with a stirrer, dropping funnel and thermometer. To this is added, rapidly, ten grams of stearyl chloride, the temperature being held below 30° C. during the addition. 30 grams of a tetrachloroethane solution containing 39% of coumarone are admixed with 25 cc. of tetrachloroethane and this solution added to the stearyl chloride and aluminum chloride over a period of three hours keeping the temperature at about 20° C. to 30° C. The temperature is then maintained at 45° C. to 50° C. for about one hour. The reaction mixture comprising an aluminum chloride complex is then decomposed on ice and the solvents removed by steam distillation. The product is dissolved in ether and the ether solution dried with anhydrous sodium sulfate. The ether is then removed by distillation under a vacuum.

25. In precisely the same manner other acylated coumarones are prepared as more fully disclosed in the aforesaid application.

30. The final product is semi-solid and plastic, 35 and resinous in character. It dissolves readily in mineral oils in proportions used for pour point depressing.

35. We shall now indicate by way of example how our products function when added to lubricating oils.

40. In the following examples the oils designated as 1, 2 and 3 are three different kinds of lubricating oils in common commercial use. The examples also indicate the pour point of the original oil and the pour point of the oil after the addition of our pour point depressors.

*Example 1*

45. A compound prepared from 12 parts of a partially polymerized coumarone resin and 30 parts of stearyl chloride is used. The results are given in the following table showing the effect of adding 0.5% of this compound:

| 55 | Oil | Saybolt viscosity at 100° F. | Pour point, ° F. |         |
|----|-----|------------------------------|------------------|---------|
|    |     |                              | Original         | Treated |
|    |     | Seconds                      |                  |         |
| 60 | 1.  | 266                          | +30              | -15     |
|    | 2.  | 433                          | +10              | -15     |
|    | 3.  | 366                          | -5               | -15     |

*Example 2*

65. 0.5% of a product prepared from 12 parts of coumarone and 30 parts of oleyl chloride is added giving the following results:

| 70 | Oil | Saybolt viscosity at 100° F. | Pour point, ° F. |         |
|----|-----|------------------------------|------------------|---------|
|    |     |                              | Original         | Treated |
|    |     | Seconds                      |                  |         |
| 1. |     | 266                          | +30              | -15     |
| 2. |     | 433                          | +10              | -15     |
| 3. |     | 366                          | -5               | -15     |

*Example 3*

0.5% of a product prepared from 20 parts coumarone and 30 parts of stearyl chloride is added to the oils with the following results:

| Oil | Saybolt viscosity at 100° F. | Pour point, ° F. |         |
|-----|------------------------------|------------------|---------|
|     |                              | Original         | Treated |
|     | Seconds                      |                  |         |
| 1.  | 266                          | +30              | -15     |
| 2.  | 433                          | +10              | -15     |
| 3.  | 366                          | -5               | -20     |

*Example 4*

0.5% of a product prepared from 30 parts of coumarone and 20 parts of stearyl chloride is added to the oils with the following results:

| Oil | Saybolt viscosity at 100° F. | Pour point, ° F. |         |
|-----|------------------------------|------------------|---------|
|     |                              | Original         | Treated |
|     | Seconds                      |                  |         |
| 1.  | 266                          | +30              | -20     |
| 2.  | 433                          | +10              | -15     |
| 3.  | 366                          | -5               | -15     |

*Example 5*

0.5% of a product prepared from 30 parts of coumarone and 30 parts of stearyl chloride is added to the oils with the following results:

| Oil | Saybolt viscosity at 100° F. | Pour point, ° F. |         |
|-----|------------------------------|------------------|---------|
|     |                              | Original         | Treated |
|     | Seconds                      |                  |         |
| 1.  | 266                          | +30              | -10     |
| 2.  | 433                          | +10              | -5      |
| 3.  | 366                          | -5               | -15     |

*Example 6*

0.5% of a product prepared from 11.8 parts of coumarone and 30 parts of linolenyl chloride is added to the oils with the following results:

| Oil | Saybolt viscosity at 100° F. | Pour point, ° F. |         |
|-----|------------------------------|------------------|---------|
|     |                              | Original         | Treated |
|     | Seconds                      |                  |         |
| 1.  | 266                          | +30              | -5      |
| 2.  | 433                          | +10              | -15     |
| 3.  | 366                          | -5               | -15     |

Thus from the above examples it is apparent that our pour point depressors are markedly effective for the purpose intended, a pour point lowering of as much as 50° F. being obtained. Our pour point depressors are especially effective on oils having rather high pour points, thus indicating the marked ability of our compounds to prevent crystallization of the wax.

Similar results are obtained when other fatty acid chlorides having twelve or more carbon atoms are used. The amount of pour point depressor can vary over wide limits. Noticeable improvement in pour point lowering is obtained when only 0.1% of our products is added. Larger amounts, up to 2% or 3% can also be added but much greater amounts, such as 10% or 15% are not necessary in order to obtain a substantial pour point lowering.

In addition to the property of lowering the pour point of the mineral oils these products also

decrease the heat generated during running friction. The oils were tested in an apparatus described by Ralston, Hoffman and Stephens, found in National Petroleum News, dated November 3, 1937. The following table shows the temperature rises after one hour for various treated and untreated oils. In the case of the treated oils 0.5% of the product described and used in Example 1 is added.

| Oil | Description                 | Temperature rise °F. (after 1.5 hrs.) |         |            |
|-----|-----------------------------|---------------------------------------|---------|------------|
|     |                             | Original                              | Treated | Difference |
| 1   | S. A. E. 20 lubricating oil | 100                                   | 72      | 28         |
| 2   | S. A. E. 30 lubricating oil | 90                                    | 75      | 15         |
| 3   | Gas oil                     | 99                                    | 76      | 23         |

0.5% of the product lowered the pour point of the gas oil from 65° F. to 15° F.

In the appended claims we use the language "a coumarone" to include the coumarone dimers, trimers or tetramers as well as coumarone itself since the coumarone thereof is the essential polymerizing component.

Although we have referred more particularly to the use of our acylated coumarone materials with lubricating oils it is apparent that they can also be added to lubricating greases where it is desirable to reduce the heat of friction or to prevent the grease from assuming a relatively hard, non-flowing state when subjected to a cold environment. When preparing such greases we can first dissolve the pour point depressor in the

lubricating oil and then make a lubricating grease therefrom in the usual way.

Having thus described our invention, what we claim is:

1. A mineral oil containing, as a pour point depressor, an acylated coumarone, the acyl group having at least twelve carbon atoms. 5

2. A mineral oil containing, as a pour point depressor, a stearylated coumarone.

3. A mineral oil containing, as a pour point 10 depressor, an acylated coumarone polymer wherein the acyl group contains at least twelve carbon atoms.

4. A mineral oil containing, as a pour point depressor, a stearylated coumarone polymer. 15

5. A mineral oil containing, as a pour point depressor, the product obtained by reacting coumarone with a fatty acid chloride having at least twelve carbon atoms in the presence of an acylating catalyst, and recovering a catalyst-free 20 product.

6. A mineral oil containing, as a pour point depressor, the product of reacting a coumarone with stearyl chloride in the presence of an acylating catalyst and recovering a catalyst-free 25 product.

7. The process of depressing the pour point of a mineral oil which comprises adding to the oil the products resulting from reacting a coumarone with a fatty acid chloride having at least twelve 30 carbon atoms in the presence of an acylating catalyst and recovering a catalyst-free product.

ANDERSON W. RALSTON. 35  
EVERETT J. HOFFMAN.